

## UNITED STATES PATENT OFFICE

2,372,354

HECTOGRAPH BLANKET AND METHOD OF  
PREPARING SAME

Robert C. Bour, Chicago, Ill., assignor to Ditto,  
Incorporated, Chicago, Ill., a corporation of  
West Virginia

No Drawing. Application February 13, 1942,  
Serial No. 430,743

5 Claims. (Cl. 117—35.6)

The invention relates to a hectograph blanket and method of preparing same. More particularly the invention relates to a hectograph blanket comprising a copy mass, a fibrous backing impregnated with a lacquer and an intermediate bonding layer comprising a drying oil.

In the preparation of this type of hectograph blanket, the fibrous backing sheet such as cloth or paper is impregnated with a lacquer which is allowed to dry. I have noticed that lacquers which have hitherto been used for this purpose do not prevent the drying oil from penetrating into the fiber of the cloth or paper backing. Thus the full benefit of the oil for bonding is not obtained; also the presence of the oil in the backing causes progressive and overtanning of a copy mass which comes in contact with the backing when the hectograph blanket is in the form of a roll.

An object of this invention is to provide a 20 hectograph blanket in which there is substantially no penetration of the drying oil into the lacquered backing.

Other objects and advantages of the invention will become apparent as the following detailed 25 description progresses.

In accordance with this invention, the drying oil is applied to a fibrous backing which has as a final coating lacquer containing a liquid which is compatible with the lacquer and immiscible with 30 the liquid drying oil.

In the preferred embodiment of the invention, I incorporate in the lacquer a small proportion of a high boiling hygroscopic liquid containing free 35 hydroxy groups which is compatible with the lacquer and immiscible with the drying oil.

Suitable liquids include propylene glycol, trimethylene glycol, triethylene glycol, 2-methyl, 2-4 pentanediol and glycol monohydroxyacetate.

The proportions of glycols and similar materials which may be used in the lacquer may vary 40 widely. The practical lower limits of glycol materials which will work in this invention range from about 3% on the solid content of the lacquer for a medium blown drying oil and is about 10% for a light blown drying oil. Higher amounts, of course, may be used up to the limit of compatibility with the lacquer.

The glycol may be incorporated to advantage in any lacquer which dries to a water insoluble film, but it is particularly advantageous to incorporate these materials in a cellulose ester or resin lacquer which contains a plasticizer which is compatible with a drying oil such as linseed oil.

Any type of drying oil may be used in the bond-

ing layer. One advantage of this invention is that it allows the use of thin bodied drying oils, as well as the heavy blown oils. The thin bodied drying oils such as the light and medium blown linseed oils give better bonding than the thicker drying oils but hitherto the excessive penetration of these oils into the backing has retarded their use. By this invention such penetration is prevented. Also by this invention it is possible to spread the drying oil on the backing in a thinner layer than has been customary.

The following are examples of lacquers which have been found suitable in the practice of my invention:

|                           | Parts by weight |
|---------------------------|-----------------|
| I. Nitrocellulose         | 25              |
| Glycol monohydroxyacetate | 10              |
| Butanol                   | 15              |
| Butyl acetate             | 10              |
| Ethyl acetate             | 20              |
| Toluene                   | 20              |

|                    | Parts by weight |
|--------------------|-----------------|
| II. Nitrocellulose | 25              |
| Propylene glycol   | 10              |
| Butyl alcohol      | 15              |
| Butyl acetate      | 10              |
| Ethyl acetate      | 20              |
| Toluene            | 20              |

|                           | Parts by weight |
|---------------------------|-----------------|
| III. Nitrocellulose       | 20              |
| Castor oil                | 5               |
| 2-methyl, 2-4 pentanediol | 10              |
| Ethyl acetate             | 25              |
| Butyl alcohol             | 10              |
| Butyl acetate             | 10              |
| Toluene                   | 20              |

The lacquers given above were used to coat and impregnate a cloth backing. After drying, a coating of linseed oil was applied to one side of the lacquered backing and allowed to dry for several hours. The copy mass composition, such as an ordinary gelatin hectograph composition, was applied to the dried linseed oil to form a hectograph blanket in the manner well known to the art. This blanket was characterized by showing substantially no penetration of the drying oil into the cloth backing. Similar results were obtained with a lacquered paper backing and with drying oil bonding agents other than linseed oil.

While there have been shown and described certain embodiments of the invention, it is to be understood that it is capable of many modifica-

tions. Changes, therefore, may be made without departing from the spirit and scope of the invention as described in the appended claims, in which it is the intention to claim all novelty inherent in the invention as broadly as possible, in view of the prior art.

I claim:

1. A hectograph blanket comprising a tannable gelatinous copy mass, a fibrous backing and an intermediate bonding layer comprising a drying oil, said fibrous backing being coated with a lacquer containing a liquid selected from the group consisting of polyhydric alcohols and incompletely esterified polyhydric alcohols.

2. A hectograph blanket comprising a tannable gelatinous copy mass, a fibrous backing and an intermediate bonding layer comprising a drying oil, said fibrous backing being coated with a lacquer containing a polyhydric alcohol.

3. A hectograph blanket comprising a tannable gelatinous copy mass, a fibrous backing and an intermediate bonding layer comprising a drying oil, said fibrous backing being coated with a lacquer containing propylene glycol.

4. A hectograph blanket comprising a tannable gelatinous copy mass, a fibrous backing and an intermediate bonding layer comprising a drying oil, said fibrous backing being coated with a lacquer containing 2-methyl, 2-4 pentanediol.

5. A hectograph blanket comprising a tannable gelatinous copy mass, a fibrous backing and an intermediate bonding layer comprising a drying oil, said fibrous backing being coated with a lacquer containing glycol monohydroxyacetate.

ROBERT C. BOUR.